

## UNITED STATES PATENT OFFICE

2,230,977

SINGLE SOLUTION PHOTOGRAPHIC  
DEVELOPING AND FIXING BATH

Garnet Philip Ham, Riverside, Conn., assignor to  
American Cyanamid Company, New York, N. Y.,  
a corporation of Maine

No Drawing. Application April 4, 1940,  
Serial No. 327,782

9 Claims. (Cl. 95—88)

This invention relates to photographic baths which are combined developing and fixing solutions for silver halides.

There have been in the past sporadic attempts 5 to produce a solution which would both develop and fix silver halide photographic material. Such a product would solve a very important problem particularly in X-ray photography where a photographic bath is desired that would develop to a predetermined density and then fix so that accurate timing is not necessary. The problem of obtaining uniform reproducible density is also an important one and which could be solved by a combined developing and fixing solution which 15 would operate satisfactorily.

With one exception, the proposals in the past have been unsatisfactory as the nature of the image developed has not been satisfactory and fogging and other difficulties have been encountered.

20 A more recent development has obtained practical results. This bath is based on the use of certain reducing sugars in the combined developing-fixing solution. The best products obtained with reducing sugars do show satisfactory images 25 and give reasonably reproducible densities. The products also have satisfactory keeping qualities if not exposed to actinic light for too long a period of time. However, in spite of the fact that useful results may be obtained with combined developing and fixing baths using reducing sugars or other analogous carbohydrates, these baths 30 have been open to the very serious objection that the emulsion speed in the case of photographic negatives is greatly reduced and has to be compensated for by increased exposure or otherwise 35 under-exposed, low-density images are obtained. This is a very serious handicap for many purposes because high emulsion speed is one of the most important properties of modern negative material.

40 During investigations which led to the development of the process of the present invention, the effects of varying quantities of fixing ingredients such as sodium thiosulfate was investigated and 45 it was found that a combined developing and fixing bath could be produced merely by reducing the concentration of the thiosulfate to a very low figure of the order of magnitude of about 10%. Such baths operate effectively with clear development and fixing and adequate contrast, but they 50 were exhausted by a single use to a point where satisfactory images could not be produced.

According to the present invention, it has been 55 found that combined developing and fixing solutions can be prepared by the use of aminobenzoic

acids and their salts, particularly anthranilic acid, which show good contrast control and decreased effect on the emulsion speed. In fact, with some of the preferred baths of the present invention, there is but little or no loss in emulsion speed with many classes of negative material. The baths of the present invention are also characterized by excellent keeping qualities and by a relatively low sensitiveness to actinic light.

It is a further advantage of baths of the present invention that they do not exhaust so rapidly and therefore can be reused.

The factors of emulsion speed and rate of exhaustion are to some extent connected. Larger amounts of thiosulfate permit the re-use of the baths on larger amounts of negative material, but at the cost of somewhat increased effect on emulsion speed. The best compromise between maximum emulsion speed and minimum exhaustion of the bath will vary for different uses. Thus, for example, where a bath is going to be used only once or twice, the compromise giving maximum emulsion speed will be chosen.

It is an advantage of the present invention 25 that it is generally applicable with various types of silver halide developers. Thus, it can be used in developers which have hydroquinone as their main developing agent or in the more common metol-hydroquinone types. The different solutions will give different results depending on the 30 nature of the developing agents used as is well known in the art, and it is an advantage of the present invention that it is generally applicable to the common types of silver halide developers.

The fixer, which is a thiosulfate, may be ordinary sodium thiosulfate or it may be any of the amino-amidine thiosulfates such as guanidine sulfate or mixtures of guanidine and sodium thiosulfates which are described and claimed in the 35 U. S. patent to Barnes, No. 2,174,494. The developing and fixing solutions of the present invention may use various alkalies to bring about developing action. It is an advantage of the present invention that the ordinary alkalies may 40 be used such as sodium hydroxide, sodium carbonate, borax, borate mixtures, and the like. In many cases we have found that improved results are obtained when an amino-amidine carbonate is used either alone or admixed with other alkalies 45 such as sodium carbonate. We do not claim here the use of guanidine carbonate per se, as this has been described and claimed in the U. S. Patent 2,174,494, cited above. Good results may also be 50 obtained by using alkalies containing a quater-

nary ammonium compound such as described in U. S. Patent 2,179,790.

The invention will be described in greater detail in conjunction with the following specific examples. The parts are by weight except in the case of liquids where they are in corresponding parts by volume.

*Example 1*

10 A photographic solution was prepared as follows:

|                                            | Parts  |
|--------------------------------------------|--------|
| Water at 25° C.                            | 100.00 |
| Sodium bisulfite                           | 1.22   |
| 15 Hydroquinone (p-dihydroxybenzene)       | 1.22   |
| Potassium bromide                          | 0.50   |
| Sodium hydroxide                           | 1.30   |
| Anthranilic acid or guanidine anthranilate | 0.40   |
| 20 Sodium thiosulfate                      | 2.50   |
| Ammonium hydroxide                         | 0.50   |

The solution is made up by dissolving each component in the order as given and results in a clear, light amber colored solution with a pH value of approximately 11.00 at 25° C. and a reduction potential of -0.44 v. at 25° C., adaptable for processing films of medium photographic speed or medium X-ray film.

25 The film or plates to be processed are placed in the solution for a 10 minute period at 18° C. and then water washed for 20 minutes. The dried film or plate is comparatively free from stains and chemical fog and the surface is smooth and free from reticulation.

*Example 2*

30 A photographic solution was prepared as follows by dissolving the components in the order given.

|                                                                | Parts  |
|----------------------------------------------------------------|--------|
| 40 Water at 25° C.                                             | 100.00 |
| Metol (monomethyl-p-aminophenol sulfate)                       | 0.8    |
| Sodium sulfite, des.                                           | 4.00   |
| 45 Hydroquinone (p-dihydroxybenzene)                           | 0.50   |
| Equal mixtures of guanidine carbonate and sodium hydroxide, or | 2.00   |
| Sodium hydroxide                                               | 1.50   |
| Anthranilic acid or guanidine anthranilate                     | 0.50   |
| 50 Sodium thiosulfate                                          | 3.75   |
| Ammonium hydroxide                                             | 0.50   |

55 The solution is light amber in color, clear, and has a pH value of 11.2 at 25° C. Medium speed photographic film or plates are processed for an 8-10 minute period at 18° C., and a satisfactory negative of density less than that obtained by using the solution in Example 1, is obtained.

*Example 3*

60 A photographic solution is made up by dissolving the components in the order given below:

|                                             | Parts  |
|---------------------------------------------|--------|
| Water at 25° C.                             | 100.00 |
| 65 Metol (monomethyl-p-aminophenol sulfate) | 0.80   |
| Sodium sulfite, des.                        | 4.00   |
| Hydroquinone (p-dihydroxybenzene)           | 0.50   |
| 70 Guanidine carbonate                      | 2.70   |
| Anthranilic acid or guanidine anthranilate  | 0.50   |
| Sodium thiosulfate                          | 3.75   |

The solution prepared in this manner is al-

most water-white, clear, and has a pH value of 9.6 at 25° C. It is satisfactory for processing 35 mm. panchromatic film at 18° C. for 25 minutes which results in negatives free from stains.

*Example 4*

10 A solution is prepared as in Example 1 using 1.50 parts of guanidine thiosulfate in place of the 2.50 parts of sodium thiosulfate mentioned. The development time was 13 minutes for a medium-fast photographic emulsion and results were similar to those obtained in Example 1.

*Example 5*

15 2.5 parts of ammonium thiosulfate were used instead of the sodium thiosulfate in the formula for the solution of Example 1 and medium-fast photographic film or plates were processed at 18° C. for a period of ten minutes. Results were similar to those obtained in Example 1.

20 In the above examples guanidine anthranilate or anthranilic acid is used in preparing the combined developing and fixing solutions. The present invention, however, is not limited broadly to any particular salt of an aminobenzoic acid 25 or anthranilic acid, but I have found that particularly good results are obtained with amino-amidine salts such as guanidine anthranilate, and this is the preferred anthranilic acid salt.

25 It will be noted that in some examples anthranilic acid is added. Due to the fact that the solution as a whole is rather strongly alkaline, the anthranilic acid in the solution actually forms an anthranilic acid salt or anthranilate, and the same is true if any of the other amino 30 benzoic acids are used.

35 What I claim is:

1. A single solution silver halide developing and fixing bath comprising a silver halide developing mixture, an amino benzoate and a silver halide fixing agent.

40 2. A single solution silver halide developing and fixing bath comprising a silver halide developing mixture, an amino benzoate and a thiosulfate.

3. A single solution silver halide developing and fixing bath comprising a silver halide developing mixture, an anthranilate and a thiosulfate.

45 4. A single solution silver halide developing and fixing bath comprising a silver halide developing mixture, an amino amidine anthranilate and a thiosulfate.

50 5. A single solution silver halide developing and fixing bath comprising a silver halide developing mixture, guanidine anthranilate and a thiosulfate.

55 6. A single solution hydroquinone developing and fixing bath comprising a developing mixture containing hydroquinone, an amino benzoate and a thiosulfate.

60 7. A single solution hydroquinone developing and fixing bath comprising a developing mixture containing hydroquinone, an anthranilate and a thiosulfate.

65 8. A single solution metol-hydroquinone developing and fixing bath comprising a developing mixture containing hydroquinone and metol, an amino benzoate and a thiosulfate.

70 9. A single solution metol-hydroquinone developing and fixing bath comprising a developing mixture containing hydroquinone and metol, an anthranilate and a thiosulfate.

GARNET PHILIP HAM.